

# United States Patent [19]

[ 19 ]

Yamada et al.

[11] 3,897,254

[45] July 29, 1975

- [54] **SILVER HALIDE CONTAINING PYRAZOLONE MAGENTA COUPLER**

[75] Inventors: **Shoji Yamada; Shoichi Horii; Kiyoshi Yamashita; Kiyoshi Futaki; Mamoru Sekido, all of Nagaokakyō, Japan**

[73] Assignee: **Mitsubishi Paper Mills, Ltd., Tokyo, Japan**

[22] Filed: **May 10, 1974**

[21] Appl. No.: **468,995**

### [30] Foreign Application Priority Data

May 11, 1973 Japan..... 48-52395

- |      |                            |                 |
|------|----------------------------|-----------------|
| [52] | U.S. Cl. ....              | 96/100; 260/310 |
| [51] | Int. Cl. <sup>2</sup> .... | G03C 1/40       |
| [58] | Field of Search .....      | 96/100, 56.5    |

[56] References Cited

## UNITED STATES PATENTS

- |           |        |                      |        |
|-----------|--------|----------------------|--------|
| 2,600,788 | 6/1952 | Loria et al. ....    | 96/100 |
| 3,580,722 | 5/1971 | Sakamoto et al. .... | 96/100 |
| 3,676,137 | 7/1972 | Mizuki et al. ....   | 96/100 |

*Primary Examiner*—J. Travis Brown

*Attorney, Agent, or Firm—Cushman, Darby & Cushman*

[57] ABSTRACT

A magenta coupler having the general formula:



is conspicuously superior to the known magenta coupler in heat resistance and moisture resistance and cause little yellowing and stain of ground and moreover is high in solubility in organic solvents.

**3 Claims, No Drawings**

SILVER HALIDE CONTAINING PYRAZOLONE  
MAGENTA COUPLER

## BACKGROUND OF THE INVENTION

The present invention relates to a coupler used for the so-called protect type color photographic photosensitive materials and more particularly it concerns with color photographic photosensitive materials containing an excellent magenta coupler.

Requirements for the protect type magenta coupler being practically usable are: (1) the coupler must have excellent color forming ability and formed dye must have excellent spectral absorption properties, (2) the coupler and the dye must have fastness to moisture, heat and light and especially they must cause no discoloration of color printing paper or film while being preserved, and (3) the coupler and the dye must be highly soluble in organic solvents such as dibutyl phthalate, ethyl acetate, etc. and must not be crystallized after they are dispersed in silver halide emulsion and the dispersion is coated on a support and dried. None of the hitherto known magenta couplers have fully satisfied said requirements. For example, the following coupler disclosed in British Patent No. 680,488 has high melting point, and low solubility in a coupler solvent and the dyes obtained by color development has the absorption maximum at 545 nm to cause formation of blue-rich magenta color image and to make it difficult to reproduce bright red color.



(wherein R is an alkyl group having 4-8 carbon atoms, A is phenyl group having at least one alkyl substituents, total number of carbon atoms in said alkyl substituents being 10 or more and L is an alkylene or alkyl substituted alkylene) satisfy said requirements and color photographic photosensitive materials containing said coupler are excellent. As the alkylene indicated by L, methylene is most preferred. That is, said couplers of the present invention are superior to the known magenta couplers of 1-phenyl-3-acylamino-5-pyrazolone type in heat resistance and moisture resistance and cause little yellowing and stain of ground. In addition, the couplers of the present invention have high solubility in organic solvents such as dibutyl phthalate and ethyl acetate. The magenta color image obtained by color development using the magenta coupler of the present invention has the absorption maximum at a wavelength of 535-540 nm which is closer to short wavelength side than absorption maximum of magenta color image obtained using the known 1-(2',4',6'-trichlorophenyl)-3-acylamino-5-pyrazole and this is



## SUMMARY OF THE INVENTION

The inventors have made intensive research in an attempt to obtain excellent magenta couplers which satisfy said requirements. As the result, they have found that magenta couplers represented by the following general formula:

60

65

5

spectral absorption properties advantageous for reproduction of color. Thus, color which substantially corresponds to original color can be attained.

Amount of the coupler of the present invention added to emulsion has no special limitation, but is preferably 20-600 g per one mol of silver halide. However, the amount varies depending upon the purpose of use and is not necessarily limited to said range and may be optionally changed.

PREFERRED EMBODIMENTS OF THE  
INVENTIONTypical examples of the couplers of the present in-  
vention are as follows:

50





Examples of preparation of said compounds (1) and (2) are shown below.

<sup>45</sup> Step 2:

**Preparation EXAMPLE 1**

Preparation of the Compound (1), namely, 1-(2',4',6'-trichlorophenyl)-3-{3"-n- $\alpha$ -(2'',4'''-di-tert-amylphenoxy) butyramido-4"-n-butoxybenzamido}-5-pyrazolone

**Step 1:**

Preparation of 3-{n- $\alpha$ -(2',4'-di-tert-amylphenoxy) butyramido}-4-n-butoxy benzoic acid.

In 50 ml of dry dioxane was dissolved 3.56 g of 3-amino-4-n-butoxy benzoic acid and 1.57 g of sodium bicarbonate was added to the solution with stirring at room temperature. Furthermore, 5.76 g of n- $\alpha$ -(2,4-di-tert-amylphenoxy) butyryl chloride was added thereto and then these were stirred for 10 hours at room temperature. Undissolved materials were filtered out and filtrate was concentrated in vacuo. Hot n-hexane was added to the residue and stirred and precipitate was filtered off. This was recrystallized from methanol to obtain 4.56 g of crystal having a melting point of 148.5°-149.5°C.

**Preparation of 3-{n- $\alpha$ -(2',4'-di-tert-amylphenoxy) butyramido}-4-n-butoxy benzoic acid.**

7 ml of thionyl chloride was added to 3.38 g of 3-{n- $\alpha$ -(2',4'-di-tert-amylphenoxy) butyramido}-4-n-butoxybenzoic acid and these were refluxed for 2 hours. Excess thionyl chloride was distilled out therefrom on a water bath in vacuo and the resultant residue was used as it was for the following reaction.

<sup>55</sup> Step 3:

Preparation of 1-(2',4',6'-trichlorophenyl)-3-{3"-n- $\alpha$ -(2'',4'''-di-tert-amylphenoxy) butyramido-4-n-butoxybenzamido}-5-pyrazolone.

1.67 g of 1-(2',4',6'-trichlorophenyl)-3-amino-5-pyrazolone was dissolved in 30 ml of dry acetonitrile. To the resultant solution was added dropwise over a period of 10 minutes a solution obtained by dissolving 3.5 g of 3-{n- $\alpha$ -(2',4'-di-tert-amylphenoxy) butyramido}-4-n-butoxybenzoylchloride obtained in the step 2 in 20 ml of dried acetonitrile while refluxing and thereafter this was refluxed for 20 hours. Thereafter, acetonitrile was distilled out in vacuo and the resultant residue was

recrystallized from methylcyclohexane to obtain 2.67 g of crystal having a melting point of 120°-125°C. Elementary analysis of this crystal resulted in C:62.04%; H:6.44% and N:7.33%. (Calculated values for  $C_{40}H_{49}Cl_3N_4O_5$  were as follows: C:62.21%, H:6.40% and N:7.26%).

#### Preparation EXAMPLE 2

Preparation of Compound No. 2, namely, 1-(2',4',6'-trichlorophenyl)-3-{3"-n- $\alpha$ -(2'',4"-di-tert-  
amylphenoxy)  
butyramido-4"-n-octyloxybenzamido}-5-pyrazolone.

##### Step 1:

Preparation of 1-(2',4',6'-trichlorophenyl)-3-(4"-n-octyloxy-3"-nitrobenzamido)-5-pyrazolone.

5.57 g of 1-(2',4',6'-trichlorophenyl)-3-amino-5-pyrazolone was dissolved in 60 ml of dry acetonitrile. To the resultant solution was added dropwise over a period of 10 minutes a solution obtained by dissolving 6.9 g of 4-n-octyloxy-3-nitrobenzoylchloride in 20 ml of acetonitrile while refluxing. Thereafter, this was refluxed for 4 hours. Undissolved material in hot state was filtered off and washed with hot methanol to obtain 9.5 g of crystal having a melting point of 271°-272°C.

##### Step 2:

Preparation of 1-(2',4',6'-trichlorophenyl)-3-(4"-n-octyloxy-3"-aminobenzamido)-5-pyrazolone.

To 80% acetic acid to which 3.44 g of iron powder was added was added dropwise over a period of 20 minutes under refluxing and stirring a solution obtained by dissolving 5.56 g of 1-(2',4',6'-trichlorophenyl)-3-(4"-n-octyloxy-3"-aminobenzamido)-5-pyrazolone in 40 ml of 80% acetic acid. Thereafter, this was refluxed with stirring for 2 hours. Hot undissolved material was filtered out and filtrate was concentrated in vacuo. The residual crystal was sufficiently washed with methanol to obtain 3.84 g of crystal having a melting point of 219°-220°C.

##### Step 3:

Preparation of 1-(2',4',6'-trichlorophenyl)-3-{3"-n- $\alpha$ -(2'',4"-di-tert-  
amylphenoxy)  
butyramido-4"-n-octyloxybenzamido}-5-pyrazolone.

1.58 g of 1-(2',4',6'-trichlorophenyl)-3-(4"-n-octyloxy-3"-aminobenzamido)-5-pyrazolone was dissolved in 15 ml of dry acetonitrile. While refluxing, to the resultant solution was added dropwise over a period of 10 minutes a solution obtained by dissolving 1.22 g of n- $\alpha$ -(2,4-di-tert-amylphenoxy)-butyryl chloride in 15 ml of dry acetonitrile. Thereafter, this was refluxed for 11 hours, acetonitrile was distilled out in vacuo and the residue was recrystallized from methylcyclohexane to obtain 1.28g of crystal having a melting point of 121.0°-123.5°C. Elementary analysis of thus obtained crystal resulted in C:64.08%, H:7.09% and N:6.66%. (Calculated values were C:63.80%, H:6.94% and N:6.76% for  $C_{44}H_{57}Cl_3N_4O_5$ ).

The following Examples prove that the coupler of the present invention has high solubility in organic solvents such as dibutylphthalate and ethyl acetate, shows little yellowing due to light, moisture and heat and that dyes formed by color development have excellent spectral absorption properties.

#### EXAMPLE 1

An emulsion was prepared in such a manner that molar ratio of silver halide and coupler was 2:1 and the emulsion was coated on a under coated polyester film and dried to obtain a photosensitive material. The coating amount was such that the coupler was coated in an amount of  $3.3 \times 10^{-3}$  moles/m<sup>2</sup>. Dibutylphthalate was used as a solvent for the coupler and a mixed solvent of ethyl acetate and dimethylformamide was used as an assistant solvent. The resultant photosensitive material was exposed and then developed with a developer of the following compositions for 6 minutes.

|    |                                                                                            |        |
|----|--------------------------------------------------------------------------------------------|--------|
| 15 | Sodium hydroxide                                                                           | 1.65 g |
|    | Sodium metaphosphate                                                                       | 50 g   |
|    | Sodium sulfite anhydrous                                                                   | 1.8 g  |
|    | Potassium bromide                                                                          | 0.5 g  |
| 20 | 4-Amino-N-ethyl-N-( $\beta$ -methanesulfonamidoethyl)-m-toluidinesesquisulfate monohydrate | 4.4 g  |
|    | Sodium hexamethaphosphate                                                                  | 0.5 g  |
|    | Hydroxylamine hydrochloride                                                                | 1.0 g  |
|    | Benzyl alcohol                                                                             | 24 ml  |
|    | Diethylene glycol                                                                          | 10 ml  |
| 25 | Water to make 1 l                                                                          |        |

Then, the developed photosensitive material was bleach-fixed with a Ferric salt of EDTA bleach fix of the following compositions for 4 minutes.

|    |                                    |      |
|----|------------------------------------|------|
| 40 | Ferric salt of EDTA                | 56 g |
|    | Sodium salt of EDTA Dibasic        | 2 g  |
|    | Ammonium thiosulfate               | 60 g |
|    | Sodium sulfite anhydrous           | 20 g |
|    | Sodium phosphate dibasic anhydrous | 12 g |
|    | Sodium bisulfate                   | 5 g  |
|    | Water to make 1 l                  |      |

Then, the fixed photosensitive material was washed with water for 8 minutes and thereafter was dipped in a solubilizing bath for 3 minutes and dried.

Spectral absorption curve of thus obtained magenta color image was obtained with a spectrophotometer (UV-200 manufactured by Shimazu Seisakusyo K.K.). The results are shown in Table 1. As comparative couplers, the following were employed: the known coupler 1-(2',4',6'-trichlorophenyl)-3-{3"-n- $\alpha$ -(2'',4"-di-tert-  
amylphenoxy)butyramido-4"-methoxybenzamido}-5-pyrazolone [Compound (6)]; 1-(2',4',6'-trichlorophenyl)-3-{3"-n- $\alpha$ -(2'',4"-di-tert-  
amylphenoxy)butyramido-4"-methoxybenzamido}-5-pyrazolone [Compound (7)]; 1-(2',4',6'-trichlorophenyl)-3-{3"-n- $\alpha$ -(2'',4"-di-tert-  
amylphenoxy)butyramido-4"-chlorobenzamido}-5-pyrazolone [Compound (8)]; and 1-(2',4',6'-trichlorophenyl)-3-{3"-n- $\alpha$ -(2'',4"-di-tert-  
amylphenoxy)butyramido-2"-n-butoxybenzamide}-5-pyrazolone [Compound (9)]. [The compounds (7)-(9) are couplers which are similar to the coupler of the present invention.]

Examples of preparation of said compounds



Table 1

| Compound                             | (1) | (2) | (6)* | (7)* | (8)* | (9)* |
|--------------------------------------|-----|-----|------|------|------|------|
| Absorption maximum wave length (nm). | 539 | 537 | 546  | 544  | 548  | 549  |

\*These compounds are those outside the scope of the present invention.

As is clear from Table 1, the magenta color images obtained using the couplers (1) and (2) of the present invention had wave lengths of absorption maximum which were shorter than those of magenta color images obtained using the comparative couplers (6), (7), (8) and (9). This fact proves that use of the coupler of the present invention can reproduce bright red color.

### EXAMPLE 2

Photosensitive materials produced in the same manner as in Example 1 which were not exposed to light, but were subjected to developing treatments similar to Example 1, and then to test for yellowing due to light and humid heat to obtain the results as shown in Table 2. The numerical values in Table 2 represent increment of absorption intensity to blue light. As a comparative coupler, the known 1-phenyl-3-{3'- $\alpha$ -(2'',4''-di-tert-amylphenoxy) acetamidobenzamide}-5-pyrazolone [Compound (10)].

5

solubility was expressed by amount (ml) of ethyl acetate required for dissolving 1 g of the couplers at room temperature.

Table 3

| Compound | Melting point  | Solubility |
|----------|----------------|------------|
| (1)      | 120.0°-125.0°C | 0.5        |
| (2)      | 121.0°-123.5°C | 0.5        |
| (6)*     | 134.0°-136.0°C | 1.0        |
| (7)*     | 232.0°-233.5°C | 40         |
| (8)*     | 222.0°-223.0°C | 27         |
| (9)*     | 165.5°-166.5°C | 4.0        |

\*These compounds are those which are outside the scope of the present invention.

10

15

20

25

30

The couplers (1) and (2) of the present invention had lower melting points and higher solubilities in ethyl acetate and in dibutyl phthalate than the comparative couplers. When the compounds (1) and (2) were used in photosensitive materials in the same manner as in Example 1, no crystals were separated. Furthermore, when these were dispersed in emulsion and were subjected to experiment on change with lapse of time under severe conditions, no crystals were separated and viscosity was not increased.

What is claimed is:

1. A silver halide photographic emulsion comprising a silver halide and a magenta coupler having the following general formula:



Table 2

| Compound | After exposure to sun light for 2 weeks |  | After being maintained at a humidity of 80% and at 50°C for 1 month |  |
|----------|-----------------------------------------|--|---------------------------------------------------------------------|--|
|          |                                         |  |                                                                     |  |
| (1)      | 0.06                                    |  | 0.15                                                                |  |
| (10)*    | 0.28                                    |  | 0.68                                                                |  |

\*This compound is one which is outside the scope of the present invention.

60

65

As is clear from Table 2, the photosensitive material containing the coupler of the present invention was stable to light and humid heat, caused little yellowing and coloration of ground.

### EXAMPLE 3

Melting point and solubility of couplers (1) and (2) of the present invention and of the comparative couplers used in the Example 1 are shown in Table 3. The

wherein R is an alkyl group having 4-8 carbon atoms, A is phenyl group having at least one alkyl substituent, the total number of carbon atoms in said substituents being at least 10 and L is an alkylene or alkyl substi-

tuted alkylene.

2. A silver halide emulsion according to claim 1 wherein the magenta coupler is selected from the followings:



15



16



3. A color photographic sensitive material comprising a support having thereon a layer of the silver halide

emulsion of claim 1.

\* \* \* \* \*

35

40

45

50

55

60

65